

April 30, 1957

T. H. ROBERTSON ET AL

2,790,698

PROCESS OF REMOVING IMPURITIES FROM FRESH SPUN  
POLYACRYLONITRILE GEL FILAMENTS BY DIRECTING  
INERT GAS BUBBLES AGAINST THE FILAMENTS

Filed Dec. 9, 1953



INVENTORS  
THOMAS H. ROBERTSON,  
PERCIVAL W. CUMMINGS, JR.

BY

*James F. Snowden*  
ATTORNEY

**PROCESS OF REMOVING IMPURITIES FROM FRESH SPUN POLYACRYLONITRILE GEL FILAMENTS BY DIRECTING INERT GAS BUBBLES AGAINST THE FILAMENTS**

Thomas H. Robertson, Stamford, and Percival W. Cummings, Jr., Cos Cob, Conn., assignors to American Cyanamid Company, New York, N. Y., a corporation of Maine

Application December 9, 1953, Serial No. 397,161

7 Claims. (Cl. 8—137.5)

This invention relates to an improved continuous process for extracting soluble material from a permeable article moving through a liquid bath.

Continuous countercurrent extraction methods have long been employed in the manufacture of various artificial and synthetic fibers by wet spinning processes. In these the coagulated filaments have been passed through one or more baths containing a solvent miscible with the solvent employed in the spinning solution or in the coagulating bath in order to free the coagulated article from the residual spinning solvent or coagulant.

An increase in the efficiency of these extractions is highly desirable in order to reduce the quantity of wash liquid required, the power required for pumping such liquid and the size of the extraction tanks. Where it is possible to recover the spinning solvent or coagulating liquid, an improved extraction process is doubly desirable in reducing the cost of the concentration or recovery of such materials from the wash liquid and in minimizing the quantity of solvent or coagulant required for make-up.

An object of the invention is to provide an improved method for extracting substances from a shaped permeable article containing extractables.

Another object of the invention is to provide an improved method of extracting liquids from gelatinous films or filaments produced by the wet spinning of a solution of polymeric material.

Other objects of the invention will be apparent to those skilled in the art from the detailed description hereinbelow.

It has been discovered that extraction efficiency is remarkably improved by directing the bubbles of an inert gas against the surface of a shaped permeable article moving continuously through a liquid extraction medium. In a specific aspect of the invention, streams of air bubbles are directed against strands of gel filaments comprising polymeric acrylonitrile containing an aqueous sodium thiocyanate while those strands are moving continuously through an aqueous bath.

It is difficult to obtain thorough extraction of processing material or other foreign substances from a continuous shaped gelatinous or other permeable article without using excessive amounts of extractant and thereby producing an extract so dilute that the cost of recovering the foreign substances is high, and sometimes not economically justifiable. Nevertheless, substantially complete removal of processing materials from the gel is often necessary to obtain certain required physical characteristics or properties in the final article. When the obvious expedient of increasing the volume of wash liquid is employed to reduce the concentration of foreign matter in the final article, the extraction process becomes distinctly less favorable from an economic standpoint. Various expedients were tried with little or no success to reduce the necessary volume of wash water while maintaining the same degree of extraction used in extracting spinning solvent from a polymeric acrylonitrile tow or strand of filaments in gel form intended for the manufacture of

staple fiber. In one of these experiments, two of a series of six wash troughs were mounted on flexible supports and the troughs were shaken bodily by means of motor-driven eccentric drives while the tow was passing there-through. In another trial, the wash liquor in one of the baths was recirculated to the same bath by means of a pump at a 140% recirculation rate (1.4 gallons recirculation per a gallon of fresh liquid introduced into the tank) with the liquid reintroduced through a fan-shaped distributor having a  $\frac{1}{16}$  inch slotted orifice directing the liquid against the tow strands from beneath in order to agitate them. The minor improvement in extraction efficiency was found to be insufficient to justify the pumping costs.

In view of the failure of simple agitation and a liquid jet to achieve the desired result, it is surprising that it can be accomplished by a mere stream of bubbles of air or other inert gas. The reasons why the stream of bubbles produces such striking effects are not fully known, but it is thought that the bubbles bring more or fresher extracting solvent into contact with the material to be extracted. However, it is apparent that the process is a physical rather than a chemical one since there are no temperature changes or differences in the final product which suggest that a chemical reaction has taken place.

The process described hereinbelow is applicable to the extraction by means of a suitable solvent or extractant liquid of any soluble material in either solid or liquid form from a continuous or substantially endless multi-filament, monofilament, film, rod, tube or other shaped article moving continuously through and beneath the surface of the extractant liquid. Although this process is especially suitable for the extraction of spinning or coagulating liquids from gelatinous polymeric materials and particularly those in the form of artificial filaments useful in textiles, it is to be understood that the novel process is operative with any continuous shaped permeable article containing extractables.

The air bubbles may be supplied from any suitable apparatus including orifices located in pipes or channels or orifices distributed along the bottom of the wash tank. In another variation the air may be bubbled through porous discs or plates of any suitable materials, including refractories and porous powdered metal structures, instead of simple holes or orifices. For example, the entire wash tank may be provided with a false bottom constructed of one of these porous materials to provide streams of bubbles through the entire area of the tank, or porous discs or strips may be inserted in pipes or other channels.

Any gas may be employed in the present process provided that it is inert, that it does not react with either the shaped article or the extraction medium and further is no completely soluble in the wash liquid at the temperature used. In general, it is recommended that a gas be selected which is not soluble to more than a small extent in the liquid medium. Air is, of course, preferred for any extraction operation in which it fits these requirements because of its low cost and ready availability.

For a better understanding of the nature and objects of this invention, reference should be had to the accompanying drawing in which the figure is a perspective view of an extraction operation according to the present invention.

The wash trough 2 has inside dimensions of approximately 12.5 feet in length and 15 inches in width. The aqueous extraction solvent for bath 4 is introduced through pipe 6 and overflows through outlet pipe 8 which is positioned to provide a bath about 9 inches deep. In this bath are located the rolls 10 and 12 which are mounted in suitable journals of known construction (not shown) and which are desirably positively driven by suit-

able conventional means. In addition air under slight superatmospheric pressure is supplied through a vertical line 14 to a horizontal distributor pipe 16 which is disposed across the width of the bath with its upper face located approximately 4 to 6 inches below the surface of bath 4. The upper face of pipe 16 is perforated with a plurality of orifices 18, for example 36 in a distance of 12 inches, of relatively small diameter as, for example, one-sixteenth of an inch or one-thirty-second of an inch, or even smaller. One or more multifilament strands 20 of an acrylonitrile copolymer fiber in the coagulated swollen gelatinous state passes downward into the bath under roll 10 and then through the length of the bath to roll 12 around which it passes before emerging from the bath for further processing elsewhere. While the strands 20 are passing through the bath air or another inert gas is being emitted from the orifices 18 in pipe 16 under slightly superatmospheric pressure to form streams of small bubbles. The fine bubbles of gas rising through the extraction bath are thus directed against the strands 20 to produce the effects described herein.

Excellent extraction results have been obtained with rolls 10 and 12 so located to position the strands 20 about 1.5 to 2 inches beneath and parallel to the surface of the bath 4. Accordingly, orifices 18 are about 2 to 4 inches below the strands. Since there is reason to believe that relatively small bubbles, ranging from those barely visible upward in size to about 0.3 inch diameter, provide greater extraction efficiency than is realized with larger bubbles; the holes 18 should not be located unnecessarily far below the strands 20. There is a tendency for the bubbles to coalesce into larger bubbles as they rise through the liquid, hence the greater the distance the bubbles travel the greater the opportunity for them to form larger bubbles. In general it is recommended that the orifices should be located between about 2 and between about 6 inches below the gelatinous article which is being subjected to extraction, the optimum for each particular extraction can be readily determined by experiment. Where desired more than one bubbling device 16 may be located in each extraction tank to further increase the extraction efficiency in that tank. In a 6-stage extraction operation using 6 tanks similar to trough 2, it has been found that a gas bubbling device 16 will increase the extraction efficiency at any stage in such processes. It will be noted that the strands 20 move through the tank 2 in a direction countercurrent to the flow of the extraction medium. For maximum extraction efficiency, the gelatinous fiber to be washed should be passed through the tanks in sequential order while water or other fresh extraction medium is introduced first into the sixth tank, then into the fifth tank, and thereafter into the fourth tank, countercurrently to the movement of the gelatinous strands.

Although the process of the present invention is especially adapted for the extraction of multifilament tow prepared from polymeric acrylonitrile, that is homopolymers or copolymers of acrylonitrile with compatible ethylenic monomers such as 2-methyl 5-vinyl pyridine, other vinyl pyridines, methyl acrylate, vinyl acetate, vinyl chloride, etc., according to the processes described in U. S. Patents Nos. 2,558,730 to 2,558,735 inclusive; it is to be understood that the present extraction process is not limited to these particular polymers or to filamentary materials alone. In brief, the process of the aforesaid patents entails spinning a solution of polymeric acrylonitrile with a molecular weight of about 75,000 (Staudinger) dissolved in concentrated aqueous sodium thiocyanate into a relatively dilute 10% aqueous sodium thiocyanate solution which is maintained at a temperature of approximately 0° C. The distended gel filaments must be thoroughly extracted to remove substantially all of the thiocyanate solution in order to produce a fiber of satisfactory physical characteristics for textile uses. It is also contemplated that the instant process is suitable for use in conjunction with any wet-spinning or wet-co-

agulation operation of a continuous nature as exemplified by the manufacture of both viscose and cuprammonium rayon, the manufacture of cellophane and other film or sheet materials as well as the wet-spinning of solutions of polyacrylonitrile in other known spinning solvents. The rate of bubbling a gas against the coagulated shaped article has been found to be significant in connection with extraction efficiency. In extracting solvent from tow prepared according to the process of the aforementioned patents with strands having 2330 filaments each of about 20 denier in the swollen gelatinous state (3 denier in the finished fiber), it appeared that air velocities as low as 0.1 foot per second at the orifice provide appreciable improvement over conventional extraction; however the air velocities above about 0.2 foot per second are recommended and the best results are obtained with orifice air velocities above about 1.0 foot per second. It is thought that the optimum air rate will vary for different articles in the present process. For instance, it is to be expected that a film or a comparatively thick monofilament will each have a different optimum air rate than that of a multifilament strand. Also it is likely that the permeability or gel structure of the product and probably also the chemical composition will affect the optimum air rate. Accordingly, it seems undesirable to attempt to precisely define the over-all range of suitable air velocities except for the generality that the orifice air velocity may range from about 0.1 foot per second up to velocities approaching the point at which damage to the article commences. In the case of the aforementioned polymeric acrylonitrile tow, the air rate was increased until the strands of tow were being lifted clear of the bath without damage to the fibers. The optimum air velocities at the orifice can readily be determined in each individual case by simple experimentation; thus those skilled in the art will have no difficulty in ascertaining the proper amount of air to be employed.

The tremendous improvement in extraction efficiency obtainable by the process of the present invention is evident from the results set forth in the table below which sets forth results secured with apparatus of the type described herein in extracting sodium thiocyanate solution from a copolymer of 95% acrylonitrile and 5% methyl acrylate prepared according to the process of the patents mentioned earlier.

TABLE  
Extraction of sodium thiocyanate solvent from polymeric acrylonitrile tow

| Run No.                                                            | 1     | 2        | 3     | 4     |
|--------------------------------------------------------------------|-------|----------|-------|-------|
| Tow Speed, Meters/minute                                           | 81.5  | 81.5     | 81.5  | 95.0  |
| Production Rate, Pounds fiber/hour                                 | 31.5  | 31.5     | 31.5  | 36.5  |
| Wash Water Flow Rate:                                              |       |          |       |       |
| Gallons/minute                                                     | 7.0   | 1.8      | 1.8   | 1.8   |
| Gallons/pound fiber                                                | 13.5  | 3.38     | 3.38  | 2.93  |
| Air Bubbling:                                                      | None  | Yes      | Yes   | Yes   |
| Estimated Air Rate, feet/second (4 <sup>2</sup> diameter orifices) |       | 0.5      | 0.5   | 0.5   |
| Tow Strands Separated                                              | Yes   | Yes      | No    | No    |
| Average Residual NaCNS on Tow Bone Dry Fiber Basis, percent:       |       |          |       |       |
| Tow Leaving:                                                       |       |          |       |       |
| Coagulation Bath                                                   | 155.0 | 159.3    | 143.2 | 162.0 |
| Trough No. 1                                                       | 58.8  | 54.7     | 57.7  | 91.2  |
| Trough No. 2                                                       | 29.3  | 30.9     | 28.5  | 44.0  |
| Trough No. 3                                                       | 16.5  | 6.2      | 7.6   | 14.4  |
| Trough No. 4                                                       | 8.5   | 1.4      | 1.8   | 2.8   |
| Trough No. 5                                                       | 6.6   | 0.28     | 0.39  | 0.55  |
| Trough No. 6                                                       | 4.9   | No trace | 0.10  | 0.03  |

In run 1 above using a conventional countercurrent extraction procedure for purposes of comparison, it will be observed that the tow still contained approximately 5% sodium thiocyanate after passing through 6 extraction baths. When the air bubbling technique was employed in runs 2, 3, and 4, the residual sodium thiocyanate was decreased at least about 98% to 0.10% or less using only about 1/4 of the volume of wash water employed in

run 1 under otherwise similar conditions. It is also noteworthy that the 5 strands of tow were not separated in runs 3 and 4, but were passed through the baths as a single broad band containing about 11,650 individual filaments to pose a more difficult extraction test. The comparison is even more striking in run 4 when it is noted that the speed of tow through the baths was increased more than 15% without impairing the extraction efficiency even though the wash water flow was maintained at the same total rate as in runs 2 and 3.

Since variations and modifications can be made in the process of the present invention without departing from the spirit of the invention, it is to be understood that the specific details and data set forth above are intended purely for the purpose of illustration and not to be construed in a limiting sense.

We claim:

1. A process which comprises directing bubbles composed essentially of an inert gas against the surface of a continuous fresh spun gel filament comprising a polymeric acrylonitrile impregnated with an aqueous salt solution of a spinning solvent for said polymeric acrylonitrile until some of said aqueous salt solution is removed therefrom by a physical action produced by the inert gas bubbles and while the filament is moving continuously through and beneath the surface of a liquid solvent which is inert and nonsolvent for the polymeric acrylonitrile, and is a solvent for the said aqueous salt solution.

2. A process which comprises directing bubbles composed essentially of an inert gas against a strand of a plurality of continuous fresh spun gel filaments comprising a polymeric acrylonitrile impregnated with an aqueous salt solution of a spinning solvent for said polymeric acrylonitrile until some of said aqueous salt solution is removed therefrom by a physical action produced by the inert gas bubbles and while the strand is moving continuously through and beneath the surface of a liquid solvent which is inert and nonsolvent for the polymeric acrylonitrile, and is a solvent for the said aqueous salt solution.

3. A process which comprises directing bubbles composed essentially of air against a strand of a plurality of continuous fresh spun gel filaments comprising a polymeric acrylonitrile impregnated with an aqueous salt solution of a spinning solvent for said polymeric acrylonitrile until some of said aqueous salt solution is removed therefrom by a physical action produced by the air bubbles

and while the strand is moving continuously through and beneath the surface of a liquid solvent which is inert and nonsolvent for the polymeric acrylonitrile, and is a solvent for the said aqueous salt solution.

5. A process which comprises directing bubbles composed essentially of an inert gas against a strand of a plurality of continuous fresh spun gel filaments comprising a polymeric acrylonitrile impregnated with an aqueous sodium thiocyanate solution until some of said sodium thiocyanate solution is removed therefrom by a physical action produced by the inert gas bubbles and while the strand is moving continuously through and beneath the surface of an aqueous medium which is inert and nonsolvent for the polymeric acrylonitrile, and which is a solvent for the sodium thiocyanate solution.

10. A process which comprises directing bubbles composed essentially of air against a strand of a plurality of continuous fresh spun gel filaments comprising a polymeric acrylonitrile impregnated with an aqueous sodium thiocyanate solution until some of said sodium thiocyanate solution is removed therefrom by a physical action produced by the air bubbles and while the strand is moving continuously through and beneath the surface of an aqueous medium which is inert and nonsolvent for the polymeric acrylonitrile, and which is a solvent for the sodium thiocyanate solution.

15. A process according to claim 5 in which the extraction operation is repeated by immersion of the strand of gel filaments in a series of baths with the aqueous medium and the strand being passed countercurrently from bath to bath.

20. A process according to claim 5 characterized by the bubbles of air being introduced into the aqueous medium from an orifice at an orifice velocity of at least 0.1 feet per second.

25. A process according to claim 5 characterized by the bubbles of air being introduced into the aqueous medium from an orifice at an orifice velocity of at least 0.1 feet per second.

#### References Cited in the file of this patent

#### UNITED STATES PATENTS

|           |                |               |
|-----------|----------------|---------------|
| 1,915,072 | Richter et al. | June 20, 1933 |
| 1,948,568 | Faber et al.   | Feb. 27, 1934 |
| 2,023,013 | Faber et al.   | Dec. 3, 1935  |
| 2,394,957 | White          | Feb. 12, 1946 |
| 2,431,956 | Moody          | Dec. 2, 1947  |

#### OTHER REFERENCES

Journal of the Textile Institute, December 1944, page A506.